

April 18, 1933.

D. T. JONES ET AL

1,904,240

MANUFACTURE OF ELECTRIC DETONATORS, PERCUSSION CAPS, AND LIKE ARTICLES

Filed Jan. 30, 1929



Fig. 1.



Fig. 2.



Fig. 3.



Fig. 4.

D. T. Jones & F. J. Moore  
INVENTORS

By: Marks & Cleaf  
A. T. S.

## UNITED STATES PATENT OFFICE

DAVID TREVOR JONES AND FREDERICK JOSEPH MOORE, OF SALTCOATS, SCOTLAND,  
ASSIGNORS TO E. I. DU PONT DE NEMOURS AND CO., OF WILMINGTON, DELAWARE,  
A CORPORATION OF DELAWARE

## MANUFACTURE OF ELECTRIC DETONATORS, PERCUSSION CAPS, AND LIKE ARTICLES

Application filed January 30, 1929, Serial No. 336,216, and in Great Britain February 2, 1928.

This invention relates to electric detonators, electric fuses and fuse heads which are fired by the passage of an electric current through a bridge wire which is surrounded by a readily inflammable material, or by the passage of an electric current through the material itself mixed with a suitable ingredient to render it conducting, and also relates to percussion caps and the like, for example friction primers for electrical firing.

The object of the invention is to provide improved or modified electric detonators, percussion caps and the like. As a result of researches, we have found that the lead salts of 2-mono-nitro-resorcin are of considerable utility in connection with electric detonators and electric percussion caps and the like, as referred to above, particularly in the latter case, as they are sensitive to percussion and friction to such a degree as to render them useful components in percussion caps and like percussion and friction primers, especially when they are prepared on certain lines.

The invention in brief consists in electric detonators, electric fuses and fuse heads as described above in which the igniting material is formed from or includes one or more lead salts of 2-mono-nitroresorcin, of which special cases are the basic, normal and acid salts.

The invention also consists in percussion caps and like percussion or friction primers containing one or more of the lead salts of 2-mono-nitro-resorcin of which special cases are the basic normal and acid salts.

The invention also consists in the improvements in the manufacture of electric detonators, percussion caps and the like, substantially as hereinafter described.

Referring to the accompanying drawing, which illustrates methods of carrying the invention into effect:—

Figure 1 is a sectional elevation of a low tension fuse head;

Figure 2 is a sectional elevation of a high tension fuse head;

Figure 3 is a sectional elevation of an electric fuse or igniter; and

Figure 4 is a sectional elevation of a modi-

fied form of electric fuse of the high tension type.

Referring to Figure 1, the low tension fuse head illustrated consists essentially of a piece of an insulating material 1 such as cardboard with a stepped end coated on both sides with a thin layer of metallic foil 2. A thin wire 3 is attached across the step, thus forming a bridge. The bridge is then covered with a readily inflammable material 4.

Referring to Figure 2, the high tension fuse head illustrated consists essentially of a piece of insulating material 1 such as cardboard with an unstepped end and coated on both sides with a thin layer of metallic foil 2. The lower end is then coated with a readily inflammable material 4 to which a conducting ingredient has been added.

Leading wires 5, 6, are then attached to the free ends of the metallic foil. Such an arrangement may be fixed in a paper tube, inserted into an ordinary detonator and secured therein by crimping or by cementing. On allowing an electric current to flow by way of the leading wires through the bridge wire, or the conducting mixture, the fuse head is ignited and the flash in turn ignites the detonator.

Referring to Figure 3, the electric fuse or igniter illustrated consists essentially of a mass of insulating material 1<sup>a</sup>, such as sulphur, wood, bitumen or rubber through which insulated conducting wires 2<sup>a</sup>, 3<sup>a</sup>, are fixed so that the bared ends protrude. A piece of bridge wire 4<sup>a</sup> is attached to the bared ends. The drawing shows the attachment carried out by means of solder 5<sup>a</sup>, 5<sup>a</sup>. The bridge wire is then embedded in the igniting material, which may be fixed to the bridge wire in a suitable manner, or be retained in a suitable container.

Referring to Figure 4, high tension electric fuses or igniters are made by omitting the bridge wire and embedding the ends of the conducting wires into the conducting material. The conducting material may be coated around the bared ends of the conducting wires, or retained in a suitable container.

The following examples illustrate how suitable lead salts of 2-mono-nitro-resorcin

55

60

65

70

75

80

85

90

95

100

may be conveniently prepared for use according to the present invention:—

*Example 1*

5 This is an example of a method of preparing a lead salt of 2-mono-nitro-resorcin, particularly for use in connection with electric detonators and the like.

To an aqueous solution of 1 gram molecule 10 of sodium mono-nitro-resorcinate containing 1.5 gram molecule of sodium hydroxide is added a slight excess of lead acetate solution. Samples precipitated at from 35° to 80° give better firing results than those precipitated at 15 lower temperatures. This example is not limited to the proportions given, for example, 0.5 grammie molecule of sodium hydroxide may be used in place of 1.5 grammie molecule mentioned in the above example. Soluble 20 salts of lead other than the acetate may also be used. The analysis of the basic lead salt prepared as described above shows a lead content of 68.9 per cent. The formula is therefore probably  $C_6H_5O_6NPb_2$ . By varying, 25 however, the proportion of sodium hydroxide and the conditions of precipitation, a basic salt may be obtained with a lead content of 71 per cent. apparently corresponding to a dehydrated form of the foregoing, and substantially the same in its behaviour.

*Example 2*

Referring particularly to electric detonators and the like, in place of the basic 35 lead salt of 2-mono-nitroresorcin there may be employed the normal lead salt or the acid lead salt (or both) of 2-mono-nitroresorcin. This normal lead salt of 2-mono-nitroresorcin containing 57.5 per cent. lead may be prepared from the previously known 2-mono-nitroresorcin by the addition of a solution 40 of lead nitrate to a solution of the sodium salt of mono-nitroresorcin, the salts being in equivalent proportions to give the normal 45 salt:  $C_6H_5O_4N.Pb$ .

*Example 3*

Referring again particularly to electric detonators and the like, according to this example the acid lead salt of 2-mono-nitroresorcin is employed. The acid lead salt of 50 2-mono-nitroresorcin containing 40.2 per cent. lead may be prepared from 2-mono-nitroresorcin by the addition of a solution of 55 lead nitrate containing acetic acid to sodium mono-nitroresorcinate, the salts being in equivalent proportions to give the acid salt:  $C_{12}H_8O_8N_2Pb$ .

*Example 4*

Referring particularly to percussion caps and the like, this illustrates a convenient method for manufacturing a suitable lead salt of 60 2-mono-nitroresorcin.

According to this example, a solution of 10

parts of 2-mono-nitroresorcin in the exact amount of sodium hydroxide to give the di-sodium salt and diluted to a volume of 500 parts is run into a solution of 22 parts of lead nitrate in 500 parts water, kept at 33-35° C. in a water bath during thirty minutes. After cooling, the precipitate which is bulky can be readily filtered off, washed with warm water, acetone and dried.

*Example 5*

Referring again particularly to percussion caps and the like, this illustrates a modified method of preparing a suitable lead salt of 2-mono-nitroresorcin.

According to this example, the precipitation of Example 4 is repeated, keeping the temperature of the mixed solutions at 63-65° C. The precipitate in this case settles rapidly, and is much denser than in Example 4.

*Example 6*

Referring again more particularly to percussion caps and the like, this is an example of four different cap mixtures by way of illustration—

|                                | Per cent |
|--------------------------------|----------|
| (a) Lead mono-nitroresorcinate | 35       |
| (of about 64% lead)            |          |
| Lead styphnate                 | 30       |
| Barium nitrate                 | 35       |
| (b) Lead styphnate             | 33½      |
| Lead mono-nitroresorcinate     | 33½      |
| (of about 57% lead)            |          |
| Pentaerythritol tetranitrate   | 33½      |
| (c) Lead mono-nitroresorcinate | 60       |
| (containing 64% lead)          |          |
| Lead styphnate                 | 40       |
| (d) Potassium picrate          | 20       |
| Barium nitrate                 | 30       |
| Lead mono-nitroresorcinate     | 50       |
| (containing 64% lead)          |          |

*General*

The normal and acid lead salts of lead mono-nitroresorcinate separately or together may be used in admixture or compounded with the basic salt, or with lead oxide, or with hydrated lead oxide, or with one another.

Particularly in the case of electric detonators and the like, the following points may be noted:—

(a) The new salts are not such powerful explosives as basic lead trinitroresorcinate. When a fuse head is ignited and the material of the flashing composition is too powerful, there is a tendency to scatter the outer dips of the fuse head instead of igniting them. The ignition of the lead salts of 2-mono-nitroresorcin is gentle, and ignites the outer dips well, giving a good flash which will initiate a detonator or fire safety fuse.

(b) The salts will not detonate when ignited even in considerable quantities, but burn

- quietly. They are therefore safer for handling than lead trinitroresorcinate.
- (c) They form a readily workable and permanent paste with the ordinary collodion used for dips in the fuse head manufacture. This paste is formed without gelatin.
- (d) They stand extreme climatic storage conditions without deterioration.
- Particularly in the case of percussion caps and the like, it is noted that the products of Examples 4 and 5, after drying, run well, and presumably consist wholly or in part of the normal lead salt of 2-mono-nitroresorcin.
- Basic and acidic salts for use in connection with percussion caps and the like may conveniently be prepared as described above.
- Any of the forms of lead salts of 2-mono-nitroresorcin may be used as the sole ingredients of percussion caps and like percussion and friction primers or admixed salts may be used.
- The invention is not limited to the methods of making these salts referred to above, nor to the compositions or proportions of these salts and other ingredients in percussion caps and like percussion and friction primers given above, but for example ingredients heretofore used in cap manufacture may be employed.
- 30 We claim—
1. Electric detonators, electric fuses, igniters and fuseheads in which the igniting material includes lead salts of 2-mono-nitroresorcin of which special cases are the basic, 35 normal and acid salts.
  2. Electric detonators, electric fuses, igniters and fuseheads as claimed in claim 1, in which a basic lead salt of 2-mono-nitroresorcin constitutes the igniting material, this 40 salt being obtained as a precipitate from a mixture of alkali salt of 2-mono-nitroresorcin and a soluble lead salt.
  3. Electric detonators, electric fuses, igniters and fuseheads as claimed in claim 1 in which normal lead salt of 2-mono-nitroresorcin constitutes the igniting material, this salt being obtained as a precipitate from an admixture of a solution of lead nitrate and a solution of an alkali salt of mono-nitroresorcin.
  4. Electric detonators, electric fuses, igniters and fuseheads as claimed in claim 1 in which an acid lead salt of 2-mono-nitroresorcin is used, this salt being obtained as a precipitate from an admixture of an alkali salt of mono-nitroresorcin with a solution of lead nitrate containing acetic acid.
  5. Percussion caps and percussion and friction primers containing a lead salt of 2-mono-nitroresorcin.
  6. Percussion caps and percussion and friction primers containing a mixture of lead salts of 2-mono-nitroresorcin, these being selected from a group consisting of basic, 65 normal and acid salts.
7. Electric detonators, fuses, igniters and fuseheads, in which the ignition material consists of acid lead salts of 2-mono-nitroresorcin.
8. Electric detonators, fuses, igniters and fuseheads, in which the ignition material consists of normal lead salts of 2-mono-nitroresorcin.
9. Electric detonators, fuses, igniters and fuseheads, in which the ignition material consists of basic lead salts of 2-mono-nitroresorcin.
10. Electric detonators, fuses, igniters and fuseheads in which the priming material consists of acid lead salts of 2-mono-nitroresorcin.
11. Electric detonators, fuses, igniters and fuseheads in which the priming material consists of normal lead salts of 2-mono-nitroresorcin.
12. Electric detonators, fuses, igniters and fuseheads in which the priming material consists of basic lead salts of 2-mono-nitroresorcin.
- In testimony whereof we have signed our names to this specification.
- DAVID TREVOR JONES.  
FREDERICK JOSEPH MOORE.